

Patented Aug. 19, 1924.

1,505,112

# UNITED STATES PATENT OFFICE.

JOSEF VON VASS, OF BUDAPEST, HUNGARY.

## APPLYING PROTECTIVE COATINGS.

No Drawing.

Application filed October 14, 1920. Serial No. 417,029.

To all whom it may concern:  
Be it known that I, JOSEF VON VASS, a subject of the Kingdom of Hungary, residing at Budapest, Hungary, have invented 5 certain new and useful Improvements in Applying Protective Coatings, of which the following is a specification.

My invention refers to protective coatings for rendering foundation pits, galleries, 10 walls and the like leak-proof, and more particularly to a method of preparing and applying coatings which are proof against liquids and acids.

It is a well-known fact that ground water, 15 and waste water (tail water) containing impurities and salts, have so detrimental an effect upon concrete constructions that concrete is avoided in tunnel and canal constructions in spite of the extraordinary advantages it offers.

All endeavours to provide concrete with a reliable insulation against the detrimental influences of ground and waste water have hitherto failed because in the majority of 25 cases it was not possible to apply the water-proof coating to the outer surface of the building, as, for instance, a tunnel or large canal, in a manner free from objections. For hitherto it was customary first to build 30 the concrete construction which was then left exposed, without any kind of protection, to the destructive influences both chemical and mechanical, of the ground water during the critical period of setting, i. e., a 35 period when it actually had the greatest need of protection, the concrete thus becoming veritably saturated with ground and waste water.

Only after having set under the most unfavourable conditions, endeavours were then made to protect the concrete by means of acid-proof and water-proof coatings. It is, however, perfectly clear that these coatings could not offer any resistance worth mentioning against mechanical influences of some strength such as water pressure in view of the fact that these coatings had to be applied to fresh, wet concrete to which they could not adhere firmly. Consequently 45 the concrete was destroyed after a short time in spite of all precautions and insulations.

According to my invention, now, these drawbacks are remedied by providing not 50 the concrete construction, but the foundation pit (trench) or gallery shaft itself with a

protective coating or layer of asphalt capable of resistance against the chemical and mechanical influences described above, whilst at the same time having constructional 60 strength and having a water-proofing effect.

The detrimental influences of ground and drain water are avoided by this means, and more especially the fresh concrete is protected during the setting period. For just 65 this protection of the fresh concrete is the most important point to be achieved on account of the fresh concrete being far more liable to detrimental influences, both mechanical as well as chemical than old concrete 70 which has already set.

In order however, to achieve this purpose, it is of importance that the asphalt or tar concrete should be applied quickly and in 75 thicker or thinner layers corresponding to the irregularities of the foundation pit, shaft or gallery, it being of great consequence that the material applied penetrate deeply into all recesses, cracks and joints, 80 thus producing a really water-proof insulation.

Asphalt or tar concrete can, however, only comply with these demands, if it is not rammed in layers, but deposited on the surface of the foundation pit, shaft or gallery, 85 in accordance with my invention, by blowing it onto the surface in question and into the cracks and joints in sprayed condition and under high pressure, after which it is still possible to fill up gaps or rubble stone 90 containing water, behind the foundation pit now closed off in a waterproof manner, with asphalt or tar concrete by forcing the liquid material into the cavities after some method 95 already known in itself.

I am aware that paints and even cement concrete and lime-mortar have already been blown onto surface under the form of sprays, however the purpose of my invention can only be achieved by means of an acid-proof 100 asphalt or tar concrete.

No method of applying such material by spraying has as yet been devised and it would scarcely be feasible to practice it with the contrivances known up to date.

In practicing my invention I may for the inst. proceed as follows:

In a receptacle fitted with a stirring device and containing two or more chambers allowing of recharging with material during working by a system of locks or gates, 110 the asphalt is mixed with the desired addi-

tional or diluting substances and then pressed by means of compressed air to a nozzle right at the place of employment through a flexible tube. In order to reduce 5 the asphalt mixture to the liquid state and maintain it thus, the receptacle may be heated by a source of heat of some suitable kind and hot compressed air may be introduced into the asphalt mixture in fine subdivision by means of perforated pipes located 10 on the bottom of the receptacle, the compressed air not only mixing the asphalt material but also heating it rapidly, rendering it liquid and feeding it to the nozzle intimately mixed, with hot air.

Before or after escaping from the nozzle, the material is preferably further also converted into spray by means of hot compressed air containing large quantities of 20 solid material such as sand and the like, admixed to it, the spray being blown onto the working surface, or into the joints and chinks thereof, respectively, under a pressure preferably amounting to about two atmospheres.

Spraying the asphalt or tar material already mixed with hot compressed air, by aid of hot compressed air containing large quantities of sand and other solid admixtures, results in the formation of a concrete, the asphalt or tar material solidifying rapidly after being blown on.

To this end the material is filled into a receptacle likewise provided with locks or gates and consisting of two or more chambers, the said receptacle being connected with the nozzle by a second hose conduit. Through this hose pipe the compressed air conducts large quantities of sand which may 40 be controlled in regard to quantity as may be desired, so that the sand meets with the liquid tar or asphalt material respectively either within, before or behind the nozzle and after having been thoroughly mixed therewith, is blown against the surface to be protected or the floor and walls respectively, of the pit or the gallery there to solidify and set.

I may, however, also proceed so as to 50 first mix the sand, clay, and other material with ground asphalt, tar or some other bituminous product in powdered condition this dry mixture then being conducted under pressure through a flexible pipe from a 55 corresponding receptacle with the aid of hot or cold compressed air to a nozzle, hot compressed air being simultaneously introduced into the nozzle in order to heat the asphalt or bituminous product added to the mixture either within, before, or after its exit from 60 the nozzle, whereupon the mixture which is now capable of settling, is blown under the form of a spray onto the working surface, where it then solidifies and forms the desired asphalt concrete.

An important feature of this method consists in the fact that the formation of the mortar takes place by the application of hot compressed gases.

However, if tar or asphalt products of 70 corresponding fluidity or suitable means of solution and dilution are employed, the heating of the tar or asphalt as well as the employment of hot compressed air can of course be dispensed with.

The granular material such as sand, ground, clay and the other admixtures can also be fed to the receptacle ready-mixed with the tar or asphalt products which may either be fluid, or viscous, or powdered, the material then being conducted to the site of work under pressure through a hose-pipe by aid of hot compressed air, sufficient heat for the formation of the concrete being gained by enlisting the collaboration of the friction caused in the hose pipe. In this case as well the material is sprayed onto the working surface through a nozzle of suitable design, owing to the compressed air expanding on leaving the nozzle and thus disintegrating the material.

This modification offers the advantage that the operator need only handle a single hose and therefore works with greater facility and reliability than in handling two hose pipes, one for granular material and one for tar, both jets meeting in the nozzle just before their exit from the same. Moreover, the necessity of continually regulating the supply of liquid material is done away with, the operator thus being enabled to pay more attention to the surface he is operating upon.

I may even mix the tar or asphalt products with clay alone, thus obtaining a very pliable product which is impervious to water and therefore particularly suitable for the insulation of tunnels and shafts, provided it be pressed in whilst in the plastic or powdered state, inasmuch as in both cases a homogeneous mass is formed which is not interrupted by layers.

Preferably powdered clay or lime, or both, or other admixtures such as fibrous materials are admixed to the sand and extraordinarily high density, strength and toughness are achieved in this manner.

It is obvious that other methods, such as for instance laying on the asphalt concrete with a trowel, or ramming and pressing it into the chinks, could never be equally successful, on account of the sprayed material being far denser, besides penetrating deeply even into the narrowest cracks and being easily kept at a uniform temperature in accordance with its particular purpose, a thing which is absolutely impossible in the case of manual labour.

In employing this method not only the final result turns out to be far superior to the results of manual work but it is actually

the only feasible method, and the cheapest one at that, for applying asphalt concrete to the external walls of the foundation pit or gallery in a reliable way and with any 5 desired thickness and moreover rapidly in such a manner as to progress with the building.

In case that an increased leak-proofness of the foundation pit or the gallery should 10 be desired, I prefer pressing asphalt or tar concrete into the chinks and cavities or—in the case of dumps—into the rubble stone, either before or after laying on the asphalt concrete, this being performed by tapping 15 the walls at the corresponding points and distances and fitting tubes into these holes, the tubes then being connected with the receptacle containing the tar or asphalt, as described above, by means of pipes or hoses 20 and by then pressing the tar or asphalt into the cavities with the aid of pumps or compressed air, after having previously blown through and warmed these cavities as far as possible with hot compressed air in order 25 to prevent the material being pressed in, from solidifying prematurely.

Corresponding to the purpose, ample 30 quantities of sand and powdered clay or other materials are also mixed with the asphalt or bitumen concrete employed for pressing in.

Obviously the novel method can be employed with equal advantage in all cases where it is desirable to lay on a thick layer 35 which is impervious to water. It is applicable in the case of walls, ceilings, tanks of all kinds, pillars and the like, and for the interior or exterior coatings of conduit-pipes, all these objects thus being protected 40 against detrimental chemical influences.

I claim:

1. The method of waterproofing surfaces 45 which consists in spraying onto the surface to be protected a mixture of plastic bituminous material and solid granular material so as to force said mixture into the surface interstices.

2. The method of waterproofing surfaces 50 which consists in spraying onto the surface to be protected a hot mixture of bituminous material and solid granular material so as

to force said mixture into the surface interstices.

3. The method of waterproofing surfaces which consists in spraying onto the surface 55 to be protected a hot mixture of bituminous material, solid granular material and compressed gas.

4. The method of waterproofing surfaces which consists in spraying onto the surface 60 to be protected a mixture of bituminous material, solid granular material and hot compressed gas.

5. The method of waterproofing surfaces which consists in spraying onto the surface 65 to be protected a mixture of asphalt, clay and hot compressed gas.

6. The method of waterproofing surfaces which consists in mixing a jet of bituminous material and hot compressed gas, and a jet 70 of solid granular material and hot compressed gas and directing the combined jets onto the surface to be protected.

7. The method of waterproofing surfaces which consists in blowing hot air into the 75 cavities and joints of a wall and then spraying onto said wall a hot mixture of bituminous material solid granular material and compressed air.

8. The method of waterproofing surfaces 80 which consists in mixing a jet of dry bituminous material and a mineral substance with a jet of hot compressed gas and directing the combined jets onto the surface to be protected.

9. The method of waterproofing surfaces which consists in spraying onto the surface to be protected a mixture of liquid bituminous material, solid granular material 90 and compressed gas.

10. The method of waterproofing surfaces which consists in injecting hot air into bituminous material, pressing the plastic mixture of bituminous material and air through a pipe, mixing it with a mixture 95 of compressed air and solid granular material and spraying the final mixture into the surface to be protected.

In testimony whereof I affix my signature.

JOSEF VON VASS.